

## UNITED STATES PATENT OFFICE

2,245,620

## BINDER FOR GLASS FIBER THREADS

Hans Steinbock, Düsseldorf-Gerresheim, Germany, assignor to Owens Corning Fiberglas Corporation, Toledo, Ohio

No Drawing. Application July 13, 1939, Serial No. 284,180. In Germany July 14, 1938

5 Claims. (CL 134—18)

In the art of making threads or strands of glass fibers and like fibers, it is well-known to bind the fibers by means of adhesives such as gutta-percha, collodium, rubber solutions, varnish, shellac, waxes or like substances. Although these adhesives have a good binding power and fully close the threads, they possess numerous disadvantages. Threads treated with the said adhesives do not lend themselves well to textile treatments, such as weaving or knitting, because their surface is not sufficiently smooth and their ability to slide is unsatisfactory. Moreover, the said adhesives either cannot be removed any more from the finished fabrics or they can only be removed therefrom by the aid of organic solvents, such as alcohol, benzine, ether, carbosulphide or the like, some of which are inflammable or explosive.

However, in many cases it is necessary to remove the binder again from the finished glass fiber products because the favorable electrical and thermal properties of the glass are more or less reduced by the said adhesives.

It is the object of the present invention to provide a binder for glass fibers and threads without the above-said disadvantages, i. e. a binder which has a high binding effect and at the same time lubricates the threads or strands and can easily be washed out without having to use inflammable solvents for this purpose.

With this object in view, the binder according to the invention consists of diluted aqueous solutions of animal, vegetable or mineral oils, fats, waxes and the like or mixtures thereof, to which a water-soluble adhesive may be added for increasing the adhesiveness of the binder.

These emulsions can be prepared in the usual manner practised in the art of making emulsions with the use of suitable emulsifying agents.

A glass fiber thread or strand sized with a binder according to the invention after the setting of the binder is well closed, soft and supple and has a brilliant, slightly fatty surface which renders it highly suited for textile treatments. The setting of the binder may be accelerated by artificial drying. The binder can be readily removed again by the common textile washing media, such as aqueous soap solutions or the like.

Some examples of binders according to the invention are composed as follows:

A

|                                                 | Parts    |
|-------------------------------------------------|----------|
| Water                                           | 80 to 90 |
| Emulsifying agent such as fatty acid sulphonate | 3 to 5   |
| Animal or vegetable oil                         | 3 to 5   |
| Yellow dextrine                                 | 5 to 10  |

B

|                       | Parts |
|-----------------------|-------|
| Special wax           | 10    |
| Wax emulsifying agent | 2     |
| Water                 | 88    |

C

|                                                 | Parts    |
|-------------------------------------------------|----------|
| Water                                           | 80 to 90 |
| Emulsifying agent such as fatty acid sulphonate | 3 to 5   |
| Animal or vegetable oil                         | 3 to 5   |
| Gelatine                                        | 3 to 5   |

D

|                       | Parts |
|-----------------------|-------|
| Special wax           | 10    |
| Wax emulsifying agent | 2     |
| Yellow dextrine       | 7     |
| Water                 | 81    |

20 The emulsions may also contain up to 5% syrup.

Without affecting the possibility of removing the binder from the finished products by washing, the binder may be given either a more pronounced binding effect or a more pronounced lubricating effect as desired in accordance with the purpose for which it is used by a proper selection of various oils or by suitably mixing oils and fats, adding waxes and using suitable emulsifying agents. Thus, various modifications and variations may be resorted to without departing from the spirit and scope of the present invention as defined in the appended claims.

Having thus described my invention, what I claim as new and desire to secure by Letters Patent is:

1. A binder for glass fiber threads and the like, consisting of a diluted aqueous emulsion containing 3 to 10% fatty acid sulphonate, 3 to 10% oil and 3 to 10% dextrine.

2. A binder for glass fiber threads and the like, consisting of a diluted aqueous emulsion containing 3 to 10% fatty acid sulphonate, 3 to 10% fats and 3 to 10% dextrine.

3. A binder for glass fiber threads and the like, consisting of a diluted aqueous emulsion containing 3 to 10% fatty acid sulphonate, 3 to 10% wax and 3 to 10% dextrine.

4. A binder for glass fiber threads and the like composed of 10% wax, 2% wax emulsifying agent, 7% dextrine and 81% water.

5. A binder for glass fiber threads and the like, comprising a diluted aqueous emulsion containing 3 to 10% emulsifying agent, 3 to 10% of emulsive substance selected from the group consisting of oil, fats and wax, and 3 to 10% dextrine.

HANS STEINBOCK.